

## UNITED STATES PATENT OFFICE

2,077,371

## SYNTHETIC DRYING OIL BODIES

Alfred E. Rheineck and Benjamin Rabin, Louisville, Ky., and James S. Long, Coopersburg, Pa., assignors to Devoe & Reynolds Co., Inc., a corporation of New York

No Drawing. Application January 21, 1935  
Serial No. 2,752

13 Claims. (Cl. 260—99.40)

This invention relates to the production of synthetic esters of fatty acids derived from natural drying oils, all of which acids have at least 16 carbon atoms.

5 Under this invention products of a great variety of natures can be produced by combining together various fatty acids in proportions not found in nature, or by combining various types, or by uniting various fatty acids with many different types of organic bases which, like the polyhydric alcohols and the sugars, are adapted to be esterified.

10 A particular phase of the invention relates to the production of esters comprising a plurality of fatty acid radicals with the molecules comprising acid chains having conjugate double bonds and also poly-unsaturated acid chains not having such conjugate double bonds. The most commonly found natural oil containing conjugate 15 double bonds is China-wood oil. Another oil also containing conjugate double bonds is oiticica, and for the purpose of this application such oils are generally referred to as "conjugated" oils and the poly-unsaturated components of their acids 20 are referred to as "conjugated fatty acids".

25 China-wood oil is recognized as having many highly valuable qualities but it also creates certain difficulties. For example, it gels easily in the kettle when heated and if used without first being heat-bodied to some extent it dries or sets to a frosted film. Various expedients have been tried for overcoming this difficulty, but all the attempts heretofore tried have been subject to more or less criticism.

30 We have found that it is possible to obtain products having the advantageous qualities of the China-wood oil compounds but free from most of their defects by making up synthetic bodies in which the characteristic conjugated fatty acids 35 such as those found in China-wood oil are combined chemically in a single molecule with other bodies of a type adapted for use in film-forming compounds but having distinctly different characteristics from the conjugated fatty acids. The 40 simplest illustration of such a synthetic body is a tri-glyceride consisting of molecules each comprising at least one conjugated fatty acid chain and at least one poly-unsaturated but non-conjugated acid chain. The third chain may be of 45 either type as desired though we have usually found it advantageous to use two of the conjugated chains and one of the non-conjugated chains. Such a product can be made by mixing together the fatty acids of a conjugated oil such 50 as China-wood oil and the fatty acids of a non-

conjugated drying oil such as linseed oil or soybean oil or fish oils or any of the other well-known types, and causing them to combine with glycerine by known processes such as heating while removing water of condensation by passing 5 a stream of inert gas through the liquid. This process produces products of value but these products can be materially improved if the fatty acids are first treated to reduce the content of saturated or mono-unsaturated acids. This may 10 be done, with China-wood acids, for example, by dissolving the acids in hot alcohol which is subsequently chilled. The desired acids, eleostearic or enriched China-wood oil acids, separate out, and after filtration, progressive removal of the 15 desired acids can be had by repeated evaporation and chilling of the solution. By using this intermediate treatment the drying qualities of the final product are appreciably improved. This concentrating step is particularly valuable with 20 the conjugated oil acids.

25 Instead of mixing the fatty acids the esterification can be conducted in steps. In this connection we have found that there is a natural tendency to form the di-glyceride as evidenced by the fact that if less than two molecules of acid are used for each molecule of glycerine a substantial percentage of uncombined glycerine will separate out on standing. This permits of a method of 30 control whereby we can be assured of having substantially an oil comprising two of the conjugated acid radicals and one of the non-conjugated acid radicals to each molecule, for we can first treat the glycerine with a sufficient quantity of eleostearic acid to produce the di-glyceride and finally add the other poly-unsaturated 35 non-conjugated acid.

40 In addition to the production of tri-glycerides of the fatty acids, our invention can also be applied to the production of many other interesting products. We have found, for example, that in producing synthetic esters of the polyhydric alcohols by the combination of the acids of drying oils, the product has improved drying qualities somewhat in proportion to the increase in 45 the number of acid chains which are combined in a secondary position. Thus we have found that the drying oil acid esters of erythritol ( $\text{CH}_2\text{OH}(\text{CHOH})_2\text{CH}_2\text{OH}$ ) has better qualities than the corresponding ester of the same fatty acid with penta erythritol ( $\text{C}(\text{CH}_2\text{OH})_4$ ). Further, the corresponding ester of mannitol (which is intended to include sorbitol) has better drying qualities than the corresponding ester of erythritol. These products have distinctly val-

able characteristics even when no conjugated acid is used, and the compounds which include the radicals of the China-wood oil acids are of especial merit.

Conversely we have found that an ester of ethylene glycol where none of the acid chains will be in the secondary position has less hardening characteristic so that a plasticizer of value can be obtained by combining with the ethylene glycol molecule one molecule of eleostearic acid from China-wood oil and one molecule of another type of fatty acid derived from either a drying oil or a non-drying oil such as castor oil. The resulting product oxidizes but does not dry 10 or set hard but remains somewhat plastic and being compatible with the films of paints and varnishes can readily be incorporated as plasticizers for these products. The proportion of such mixed ethylene glycol esters found desirable 15 in paint and varnish films may range from about 20% to about 20% of the weight of the non-volatile vehicle.

In addition to the combination of the drying oil acids with the polyhydric alcohols it is also 25 within the spirit of our invention to cause these acids to combine with other related organic bases comprising a plurality of hydroxyl groups. Thus we have made many valuable products by building up molecules comprising conjugated 30 acid radicals and other poly-unsaturated drying oil acid radicals and one of the sugars such as xylose, glucose, sucrose, dextrose, galactose, maltose, and fructose and also derivatives of sugars such as gluconic acid and related bodies 35 such as simple glucosides, mannosides, and other ethers. Also if desired the acids of the blown drying oils may be used.

The production of the esters built around a sugar molecule is not possible by direct esterification. For making these products (and also in some instances for making the esters of the polyhydric alcohols) we find it advantageous first to produce the acid chlorides of the fatty acids and then cause the desired combination 40 to take place. To accomplish this combination it is advisable as known, to have present a basic material which will combine with the released hydrochloric acid. For this purpose, we may use the cyclic tertiary amines such as pyridine or other organic bases may under some circumstances be used much as di-methyl aniline, and 45 quinoline.

According to our invention, we have also combined in a single molecule the poly-unsaturated fatty acid radicals and other bodies having valuable film-forming characteristics, in particular the acid radicals of natural resins. Thus, we have made triple glycerides of conjugated fatty acid, other non-conjugated fatty acids and the acids of ordinary rosin or copals, the resulting product being a homogeneous mass, not a mixture, adapted to be used as a varnish with or without the addition of diluent.

Using the glyceride base the proportions of the other ingredients are more or less limited if the mass is to be kept homogeneous, but this is not the case with the alcohols having a greater number of hydroxyl groups or with the sugars, where wide ranges in proportions of the various acid radicals are possible. In this connection, we may point out that where a relatively high proportion of the conjugated fatty acid radicals are to be added as acid chlorides, it is advisable to use a diluting solvent. Such a solvent may also be used with other types of poly-unsatu-

rated fatty acids but its use is not then so essential. Among the solvents which we have found useful for this purpose are isopropyl ether, chloroform, benzene, and toluene.

In order further to explain our invention we give a number of specific examples. In these, where acid chlorides are used they were prepared by treating the respective fatty acids with phosphorous trichloride. After standing at room temperature for one hour, and then heating at 100° C. for one hour, two layers separate. The clear liquid, which is the acid chloride mixture, was then poured off from the underlying brown layer. The acid chlorides are next freed from hydrochloric acid by passing a stream of 15 gas, e. g., carbon dioxide, through the warm product, until the issuing vapors no longer turn white in the presence of moisture. Various other methods of preparing acid chlorides involving phosphorus penta chloride, phosphorus oxychloride, thionyl chloride and others are known in the art and need not be here explained.

#### Example 1

The following is an example of an oil prepared 25 by the esterification of sucrose with China-wood acid chlorides and perilla acid chlorides in the presence of pyridine and benzene.

|                           | Parts | 30 |
|---------------------------|-------|----|
| Sucrose                   | 34.2  |    |
| China-wood acid chlorides | 60    |    |
| Perilla acid chlorides    | 180   |    |
| Pyridine                  | 96    |    |
| Benzene                   | 800   | 35 |

Mix the finely powdered sucrose, China-wood acid chlorides, perilla acid chlorides, and benzene, and while agitating vigorously, add the pyridine over a period of an hour. The temperature will rise to about 40° C. Pour the reaction product 40 into an equal volume of methyl alcohol. Wash the oil which separates several times with hot methyl alcohol. Drive off the excess alcohol by heating below 100° C. and passing through it a stream of carbon dioxide.

The resulting product is a viscous brownish yellow oil, which sets to a very tough non-frosting water-resistant film. It dries much more rapidly than natural drying oils, e. g., linseed, perilla, etc.

Other similar examples were run in which the China-wood acid chlorides ranged up to as much as 208 parts with a proportionate reduction of the perilla acid chlorides. In some cases the benzene was reduced to about 240 parts. Even with the high proportion of China-wood oil acids 55 the resulting oil dried to a clear, non-frosting film.

#### Example 2

The following is an example of an oil prepared 60 by the esterification of dextrose and China-wood acid chlorides and linseed acid chlorides.

|                           | Parts | 65 |
|---------------------------|-------|----|
| Dextrose                  | 18    |    |
| China-wood acid chlorides | 50    |    |
| Linseed acid chlorides    | 100   |    |
| Pyridine                  | 40    |    |
| Benzene                   | 100   |    |

Mix the dextrose, the acid chlorides, and benzene and to this mixture add the pyridine while stirring. Pour the reaction mixture into an equal volume of methyl alcohol. Wash the oily layer with methyl alcohol several times until practically 70 free from acid. Dry the oil by heating below 75

100° C. and blowing through it a stream of carbon dioxide.

The product is a fairly pale viscous oil. With driers it sets to a smooth, tough, water-resistant film.

*Example 3*

This example describes the preparation of an oil from dextrose, China-wood acid chlorides and perilla acid chlorides.

|                           | Parts |
|---------------------------|-------|
| Dextrose                  | 18    |
| China-wood acid chlorides | 110   |
| Perilla acid chlorides    | 40    |
| Pyridine                  | 40    |
| Benzene                   | 200   |

Mix the dextrose, China-wood acid chlorides, perilla acid chlorides, and 100 parts of benzene. To this mixture add while stirring a mixture of 20 pyridine and 100 parts of benzene. Purify the resulting oil as described in Example 2.

*Example 4*

This is an example of a dextrose ester having 25 all the hydroxyl groups condensed with China-wood acid residues.

|                           | Parts |
|---------------------------|-------|
| Dextrose                  | 18    |
| China-wood acid chlorides | 150   |
| Pyridine                  | 40    |
| Benzene                   | 200   |

This oil was prepared and purified exactly as described in Example 2. The product was an amber colored, viscous liquid. It dried to a soft 35 frosting film.

*Example 5*

The following is an example of an oil made by 40 condensing mannitol with China-wood acid chlorides and sardine oil acid chlorides.

|                            | Parts |
|----------------------------|-------|
| Mannitol                   | 18.2  |
| China-wood acid chlorides  | 114   |
| Sardine oil acid chlorides | 69    |
| Pyridine                   | 48    |
| Benzene                    | 120   |

The oil was prepared and purified in the same manner as the oil of Example 2. With driers it sets to a firm, water-resisting non-frosting film.

*Example 6*

The following is an example of an oil prepared by condensing pentaerythritol with China-wood acid chlorides and sunflower acid chlorides.

|                           | Parts |
|---------------------------|-------|
| Pentaerythritol           | 13.6  |
| China-wood acid chlorides | 76    |
| Sunflower acid chlorides  | 44    |
| Pyridine                  | 32    |
| Benzene                   | 40    |

This oil was prepared and purified in exactly the same manner as described in Example 2. The oil is a light-amber colored liquid.

*Example 7*

This is an example of a mixed ester of glycerol with equal parts of China-wood and perilla acid residues.

|                           | Parts |
|---------------------------|-------|
| Glycerol                  | 9.2   |
| China-wood acid chlorides | 45    |
| Perilla acid chlorides    | 45    |
| Pyridine                  | 24    |
| Benzene                   | 60    |

This oil also was prepared in the same manner as that of Example 2. It is a pale fairly fluid oil.

In another case 60 parts of China-wood acid chlorides were used with 30 parts of linseed acid chlorides.

*Example 8*

The following is an example of an oil prepared by direct esterification of glycerol with mixed China-wood linseed and rosin acids (abietic acid).

|                         | Parts |
|-------------------------|-------|
| Glycerol                | 92    |
| China-wood fatty acids  | 280   |
| Linseed oil fatty acids | 280   |
| Abietic acid            | 302   |
|                         | 15    |

Agitate and heat the reactants at approximately 210° C. until the desired acid value is obtained, generally less than 10. This usually requires about 10 hours, but can be shortened if higher temperatures are used; however, the tendency for gel formation is increased; during the process a stream of carbon-dioxide is passed through the mixture.

The resulting viscous oil sets to a tough, tenacious, and non-frosting film, with drier. This product is thermoplastic.

It is soluble in the usual varnish thinners.

*Example 9*

The following is an example of the preparation of a mixture of monoglycerides and diglycerides of perilla fatty acids.

|                     | Parts |
|---------------------|-------|
| Glycerol            | 92    |
| Perilla fatty acids | 280   |
|                     | 35    |

Follow the method outlined in Example 8. The time required to reach a negligible acid value is about four hours. Not all of the glycerol is esterified, and can easily be separated from the esters.

The product so obtained is a mixture and one batch gave the following composition on analysis.

|                | Percent |
|----------------|---------|
| Mono-glyceride | 47      |
| Di-glyceride   | 53      |
|                | 45      |

*Example 10*

The following is an example of an oil prepared by the further esterification of a mixture of a mono- and di-glycerides of perilla fatty acids with China-wood oil fatty acids.

|                                   | Parts         |
|-----------------------------------|---------------|
| Glyceride (prepared in Example 9) | 47% Mono- 500 |
| China-wood oil fatty acids        | 53% Di- 527   |

Mix the mono- and di-glycerides with the fatty acids and heat as described in Example 8, until the acid value is reduced to a low value (1.7). This required 3½ hours.

The resulting product is very light in color and possesses a high viscosity. It sets to a tough, permanent, non-frosting film in two hours, when the normal drier content is used.

*Example 11*

The following is an example of an oil prepared by further esterification of a mixture of mono- and di-glycerides of linseed oil fatty acids with China-wood oil acid chlorides in the presence of pyridine.

|                                  | Parts          |
|----------------------------------|----------------|
| Glyceride of linseed fatty acids | 53.9% Mono- 66 |
| China-wood acid chlorides        | 46.1% Di- 74.5 |
| Pyridine                         | 20             |
| Benzene                          | 200            |
|                                  | 75             |

5 Dissolve the glycerides and acid chlorides in the benzene, and add the pyridine in a slow stream and with constant agitation. Now decant the liquid from the underlying layer of separated pyridine salt and pour it into methyl alcohol. The glyceride separates immediately. The glyceride is now washed several times with methyl alcohol until neutral.

10 The product so obtained is dark in color and quite viscous. It sets to a tough, permanent non-frosting film.

*Example 12*

15 The following is an example of an oil prepared by the condensation of ethylene glycol with eleostearic acid chloride and perilla acid chlorides in the presence of pyridine.

|                           | Parts |
|---------------------------|-------|
| Ethylene glycol           | 3.1   |
| Eleostearic acid chloride | 29.8  |
| Perilla acid chloride     | 29.8  |
| Pyridine                  | 18    |

25 Agitate the ethylene glycol with the acid chlorides and add the pyridine gradually over a period of thirty minutes. The reaction mixture becomes thick and creamy. Pour the mixture into methyl alcohol, and pour off the alcohol from the insoluble layer. Wash several times with methyl alcohol to remove free acids.

30 The product is a brown viscous oil which apparently remains tough and elastic after drying and is adapted for use as a plasticizer.

*Example 13*

35 The following is an example of an oil prepared by the condensation of glycerol with the mixed acid chlorides of China-wood, perilla and rosin acids in benzene solution in the presence of pyridine.

|                           | Parts |
|---------------------------|-------|
| Glycerol                  | 92    |
| China-wood acid chlorides | 298   |
| Perilla acid chlorides    | 298   |
| Rosin acid chlorides      | 320   |
| Benzene                   | 900   |
| Pyridine                  | 240   |

40 Agitate the glycerol and acid chlorides in about one-half the quantity of benzene, and then add the pyridine, diluted with the remaining benzene, in a slow stream over a period of thirty minutes. The solution becomes thick and creamy; after standing for another thirty minutes, pour the mass into methyl alcohol; a tough 45 stringy mass separates. After several washings with methyl alcohol, a light colored viscous, clear oil separates. Several washings with the alcohol remove the free acid.

45 The oil sets to a tough clear film.

*Example 14*

50 The following is an example of an oil prepared by the condensation of pentaerythritol with rosin acid chlorides, China-wood acid chlorides and soya bean acid chlorides in benzene solution in the presence of pyridine. This corresponds to about a fifteen gallon varnish.

|                           | Parts |
|---------------------------|-------|
| Pentaerythritol           | 13.6  |
| Soya bean acid chlorides  | 29.8  |
| China-wood acid chlorides | 29.8  |
| Rosin acid chlorides      | 64.0  |
| Benzene                   | 120   |
| Pyridine                  | 35    |

Follow the method outlined in Example 13.

The product possessed a very light color, was somewhat opaque, and very viscous. It set to a tough film.

*Example 15*

5

The following is an example of an oil prepared by the condensation of mannitol with rosin, perilla, and China-wood acid chlorides in benzene solution in the presence of pyridine.

|                           | Parts |
|---------------------------|-------|
| Mannitol                  | 18.2  |
| China-wood acid chlorides | 59.6  |
| Perilla acid chlorides    | 59.6  |
| Rosin acid chlorides      | 64.0  |
| Benzene                   | 180.0 |
| Pyridine                  | 50    |

Follow the method outlined in Example 13.

The product recovered is a clear dark colored viscous oil. It set to a tough film.

*Example 16*

20

The following is an example of an oil prepared by the condensation of dextrose with rosin, China-wood, and linseed acid chlorides in benzene solution in the presence of pyridine.

|                           | Parts |
|---------------------------|-------|
| Dextrose                  | 18.0  |
| China-wood acid chlorides | 59.6  |
| Linseed acid chlorides    | 29.8  |
| Rosin acid chlorides      | 64.0  |
| Benzene                   | 150.0 |
| Pyridine                  | 40.0  |

Follow the method outlined in Example 13.

The product formed was a light colored, clear, viscous liquid, and set to a tough clear film.

*Example 17*

35

The following is an example of an oil prepared by the condensation of sucrose with rosin, China-wood and linseed fatty acid chlorides in benzene solution in the presence of pyridine. This corresponds to about a fourteen gallon varnish.

|                           | Parts |
|---------------------------|-------|
| Sucrose                   | 34.2  |
| Rosin acid chlorides      | 128.0 |
| China-wood acid chlorides | 98.4  |
| Linseed acid chlorides    | 29.8  |
| Benzene                   | 250   |
| Pyridine                  | 70    |

Follow the method outlined in Example 13.

The product is a light yellow colored, somewhat opaque, viscous oil. It sets to a tough clear film.

*Example 18*

40

The following is an example of an oil prepared by the condensation of maltose with rosin, soya bean, linseed and China-wood acid chlorides in benzene solution in the presence of pyridine.

|                           | Parts |
|---------------------------|-------|
| Maltose                   | 36.0  |
| Soya bean acid chlorides  | 59.6  |
| Linseed acid chlorides    | 89.4  |
| Rosin acid chlorides      | 32.0  |
| China-wood acid chlorides | 59.6  |
| Benzene                   | 250.0 |
| Pyridine                  | 70.0  |

Follow the method outlined in Example 13.

The product is a clear, dark colored, viscous oil which set to a tough film.

75

*Example 19*

The following is an example of an oil prepared by the esterification of alpha methyl glucoside with China-wood acid chlorides and linseed acid chlorides.

|                           | Parts |
|---------------------------|-------|
| Alpha methyl glucoside    | 21.2  |
| China-wood acid chlorides | 90.0  |
| Linseed acid chlorides    | 90.0  |
| 10 Benzene                | 90.0  |
| Pyridine                  | 50.0  |

Mix the alpha methyl glucoside with the acid chlorides and one half the quantity of benzene. Dilute the pyridine with the remaining benzene and run it into the acid chloride mixture with constant agitation in thirty minutes. Permit the creamy mass to stand for one hour and pour it into methyl alcohol. The viscous oil separates. The product is now washed several times with methyl alcohol.

It sets to a tough film.

*Example 20*

25 The following is an example of an oil prepared by condensing dextrose with the acid chlorides made from blown linseed acids.

|                                 | Parts |
|---------------------------------|-------|
| Dextrose                        | 18    |
| 30 Blown linseed acid chlorides | 150   |
| Pyridine                        | 40    |

The blown linseed acids used in this example were prepared by blowing through a stream of air through the linseed acids for 12 hours at 50° C. The blown acids were subsequently treated with  $PCl_3$  to produce the acid chloride as described previously. To a mixture of the finely pulverized dextrose and the blown linseed acid chloride add the pyridine slowly and with vigorous agitation. Wash the resulting oil with water and then several times with methyl alcohol. Drive off the residual water and methyl alcohol by heating below 100° C. and blowing through it a stream of carbon dioxide.

45 The product is a dark colored viscous oil which sets to a clear tough film.

*Example 21*

The following is an example of an oil prepared 50 by the esterification of gluconic acid with perilla oil acid chloride.

|                        | Parts |
|------------------------|-------|
| Gluconic acid          | 19.6  |
| Perilla acid chlorides | 180.0 |
| 55 Pyridine            | 50.0  |

The gluconic acid and acid chlorides were mixed and the pyridine added slowly over a period of an hour. The creamy mass was poured 60 into methyl alcohol. An oily mass, light yellow

in color, separated. The product was washed several times with methyl alcohol.

It sets to a tough film with the usual driers.

It is understood that these examples are given only by way of illustration and may be modified greatly and the steps may be combined in other combinations without departing from the spirit of our invention.

What we claim is:

1. The process of producing film-forming compounds which comprises causing an organic base having a plurality of hydroxyl groups to combine with acid radicals of a conjugated drying oil acid and of a non-conjugated poly-unsaturated drying oil acid. 10

2. A process as specified in claim 1, in which said base is a polyhydric alcohol having at least two hydroxyl groups in the secondary position.

3. A process as specified in claim 1, in which said organic base is a sugar. 20

4. A process as specified in claim 1, in which said organic base is a mono-saccharide.

5. A process as specified in claim 1, in which an acid radical derived from a natural resin is also caused to re-combine with said organic base to form a composite ester comprising at least three types of acid radical. 25

6. A process as specified in claim 1, in which the organic base is caused first to combine with acid radicals of a conjugated fatty acid present in sufficient quantity to supply at least approximately two such acid radicals for each molecule of the base. 30

7. The method of producing a plasticizer for use in film-forming compounds and the like which comprises causing ethylene glycol to react with eleostearic acid and with a natural fatty acid of a different type to produce a double ester thereof. 35

8. A drying oil consisting essentially of a compound ester of a polyhydric organic base, a drying oil acid having conjugate double bonds and a poly-unsaturated drying oil acid not having such conjugate double bonds. 40

9. A product as specified in claim 8 which comprises more than three acid radicals. 45

10. A product as specified in claim 8, in which at least one-half of the acid chains contain such conjugate double bonds.

11. A product as specified in claim 8, in which at least two of the drying oil acid radicals are combined in secondary positions. 50

12. A product as specified in claim 8, in which such ester further includes acid radicals of resin acids.

13. A drying oil consisting essentially of an ester of a sugar and the acid radicals of a blown 55 drying oil.

ALFRED E. RHEINECK.  
BENJAMIN RABIN.

JAMES S. LONG.

60